

# UNITED STATES PATENT OFFICE.

NELSON DE LONG, OF CHICAGO, ILLINOIS.

## PROCESS OF TREATING PEAT.

1,312,521.

Specification of Letters Patent. Patented Aug. 12, 1919.

No Drawing.

Application filed September 23, 1918. Serial No. 255,298.

*To all whom it may concern:*

Be it known that I, NELSON DE LONG, a citizen of the United States of America, and a resident of Chicago, county of Cook, 5 and State of Illinois, have invented certain new and useful Improvements in Processes of Treating Peat, of which the following is a specification.

My invention relates to the treatment of 10 peat so as to prepare it as a fuel or to put it in a condition for other commercial purposes. The object of the invention is to cause bog peat to give up its water content in a more expeditious and thorough manner 15 than has heretofore been possible.

Peat as it comes from the bogs normally 20 contains eighty to ninety per cent. of water. This water is largely contained in cells of the plants which give rise to peat bogs. By compression the water content may be reduced to about seventy per cent., but this is not enough to make the material useful. 25 Ordinarily air drying is a slow process and only partially accomplishes the result. Drying by heat is expensive. Furthermore, heat dried peat is friable.

Most peat is of an acid character. I have 30 discovered that by adding a small amount of alkali to the peat as it comes from the bog, the material so treated will give up its water much more freely and will dry out into the form of a hard body much resembling hard rubber in appearance and texture. The alkali used may be sodium carbonate, 35 potassium carbonate, borax, or like material. Of these I will consider sodium carbonate (commonly known as washing soda) as being typical of the class of alkalis which may be used for this purpose. Different 40 peats differ somewhat in composition and require different amounts of alkali for successful treatment, but I have found that the addition of about one-half of one per cent. by weight of sodium carbonate is satisfactory 45 for ordinary grades of peat. This soda may be added in a powdered form or may be dissolved in water and added in a liquid form.

In carrying out my process I put the peat through a mixing machine of any kind or 50 description and add the alkali to the mass while being mixed. The material is then preferably made up into blocks and left to dry in the air. A convenient way of making this material into blocks is to put 55 it through a pug mill of the kind used in making ordinary mud brick. If the peat with added alkali is treated as clay is treated in ordinary brick making and if made into two-inch cubes, it will dry out in from 60 eight to twelve days into hard blocks only a little over one inch on each side. These blocks may then be used as ordinary coal or lignite is used.

The mixed peat and alkali may be left 65 to dry in mass, but is requires longer to accomplish the drying process. With the alkali added, peat dries in air into a hard and solid body, and not into a friable body as when air dried without the addition of 70 alkali.

What I claim is:

1. The process of removing water from peat at ordinary temperatures and pressures which consists in mixing with the peat a 75 small quantity of alkali of a kind which will attack the water-holding cells of the peat without combining with the water thereof, and in exposing the mixture to the outside air. 80

2. The process of removing water from peat at ordinary temperatures and pressures which consists in mixing with the peat a small quantity of alkali which will attack the water-holding cells of the peat but will 85 not combine with the water thereof, in forming the mixture into blocks, and in drying such blocks by exposing them to the air.

3. The process of removing water from peat at ordinary temperatures and pressures 90 which consists in mixing with the peat about one-half of one per cent. by weight of sodium carbonate, and in exposing the mixture to the action of the outside air.

NELSON DE LONG.

Copies of this patent may be obtained for five cents each, by addressing the "Commissioner of Patents, Washington, D. C."